

(No Model.)

J. J. WILLIAMSON.  
COMBINING OF STEELS.

2 Sheets—Sheet 1.

No. 295,965.

Patented Apr. 1, 1884.



FIG. 1.

FIG. 2.

FIG. 3.

WITNESSES

George R. Totman  
Red. Harris

INVENTOR

J. J. Williamson  
*by his atty*  
Clarke & Raymond

(No Model.)

2 Sheets—Sheet 2.

J. J. WILLIAMSON.  
COMBINING OF STEELS.

No. 295,965.

Patented Apr. 1, 1884.



WITNESSES

George R. Totman  
John Harris

FIG. 4.

INVENTOR

J. J. Williamson  
by his atty  
Clarke & Raymond

# UNITED STATES PATENT OFFICE.

JOHN J. WILLIAMSON, OF BOSTON, MASSACHUSETTS.

## COMBINING OF STEELS.

SPECIFICATION forming part of Letters Patent No. 295,965, dated April 1, 1884.

Application filed July 22, 1882. (No model.)

*To all whom it may concern:*

Be it known that I, JOHN J. WILLIAMSON, of Boston, in the county of Suffolk and State of Massachusetts, a citizen of the United States, 5 have invented a new and useful Improvement in the Combining of Steels; and I do hereby declare the following to be a full, clear, and exact description thereof.

My invention consists in the modes and manners of combining two or more different qualities of steel of varying carbon degree of hardness, ductility, strength, and fusibility in one and the same mass, securing the relative position, perfect soundness, freedom from porosity, 15 complete homogeneity, and certain union of the various steels of which the ingot or mass is composed, so that there may be no lines of separation or of demarcation between them, securing at comparatively low cost an ingot, 20 block, slab, or mass of metal composed of a combination of the same metal varying only as to qualities and quantities, the product of which represents in part the high powers of steel—such as ability to take and maintain 25 hardness and temper, high resistance to tensile, torsional, deterrent, and crushing strains—and in addition thereto the qualities of best wrought-iron (yet in greater degree)—such as ductility, non-liability to sudden fracture, 30 with the invaluable property of welding and forging at high heats—can be treated in ordinary forge-fires and heating-furnaces without consequent liability to destruction from exposure to oxidizing flames, as certainly would 35 be the case with naked steel of high quality.

By combining the various qualities of steel “en masse,” I secure to commerce and manufacturers a new article of manufacture, which possesses within its own inherent qualities the 40 requisites desired in one and the same mass, block, or bar—such as ability to be forged at any heat, welded with ease and safety, to receive and maintain temper, stiffness, strength to great degree, with the safe factor of ductility, which represents the non-liability to fracture under either sudden or continued concussion or vibratory strains. The outer section or portion of the ingot, block, or mass of the 45 first instance is composed of the quality of metal known as “mild steel,” or, otherwise, “ingot iron,” of such grade as will enable it to

withstand the heats only by which it can be welded, and the subsequent processes of manipulation and reduction on forging either by rolls, hammer, or any process usual in “working” malleable metal of this nature. By preference, I would choose for such outer section or envelope of the ingot or mass the mild steel made by the process known as the “dephosphorizing process,” for the reasons that it can be produced more cheaply, and is believed to have greater fluidity than mild steels made by other processes at the present time. Yet I do not confine myself to the use of 55 mild steel produced by said dephosphorizing process alone, but claim as well the use of said quality of mild metal made by the Bessemer process proper or by the Siemens-Martin, or other open-hearth or pneumatic process which will produce the desired results—viz., the ability to weld in fusion and sustain forging and treatment at high heats, an ample test being “the ability of the metal to sustain without injury the heats and treatment necessary to perfect its own homogeneity.” 70

There are various modes and details of utilizing my invention, which are properly a part of it, whereby I am enabled to produce the results sought in the easiest, most reliable, and economical manner, securing commercial success and enhancing the benefits from the invention to the public. 75

By one of my methods I first cast a hollow ingot of mild steel of any form, dimensions, and thickness of mass, with one end wholly or partially closed, the other being open to enable its being filled either with molten steel or steel in scrap or ingot or bloom, or by using both solid and fluid steels—a combination of the two methods. By another method of procedure, which has its advantages, a compound ingot or mass of varying qualities of steel can be made equally well with the mode first described, first casting the ingot block or mass which is designed to form the center of the 95 final mass of such form, dimensions, and quality of metal as desired, and at any subsequent time this first or center ingot can be placed within an ordinary mold suitable for the purpose, and the second quality of metal poured 100 to it. If desired, the first or center ingot can be placed within the mold for ingot No. 2 in

such manner that the steel poured to it will envelop it completely or not, as wished. The prior ingot in any case may or may not be placed in the center of the mold for the following ingot, as the result to be gained may suggest. In the one case the following metal will be equally distributed from a center line and in the other it will not be—as, for instance, an ingot or mass of two steels being cast from which railroad-rails are to be manufactured, the center ingot being of hard steel set to one side of the center of the mold, the mild steel poured to it enveloping it but slightly on one side and heavily upon the other. The side of the ingot where the mild steel is of the lesser section represents in the finished article the head of the rail and the thick side of mild steel the base, thus securing practically a safe rail of great endurance.

20 The qualities, quantities, and relative positions of the various steels used in filling the hollow ingot of mild steel, to be determined by the desire to produce a given result: Closing the opening in the hollow ingot of mild steel by any suitable means, the whole mass is charged into a heating-furnace, and its temperature raised to the point of welding, when it is drawn and sent to the rolls or other appliances for manipulation and forging.

25 30 The treatment of the ingot or mass to the welding-heat necessary to cure its defects and insure soundness subsequent to its formation by casting and working it at such high temperatures secures, first, the perfect freedom from porosity; second, soundness of the mass in its entirety; third, removing the lines between contiguous steels and merging the varying qualities to such extent that there no longer remains a distinctiveness of quality at their junction. It is only by this subsequent treatment of the mass to the high welding temperature and the manipulation of it at that heat that a sound article can be produced from compound or composite steels. This process of casting steel upon steel can be followed or repeated in the formation of an ingot or mass as often as wished, at the convenience of the manufacturer. These ingots or masses of single or compound steels can be placed in the mold 35 for the final operation of casting round about them the envelope of mild steel, they being so situated and sustained within the mold that the molten mild steel, in pouring, incloses the mass at base and top, so that no portion of the inner mass may be presented to the flame when reheating or to the oxidizing and destructive effects of exposure when at high temperatures.

40 45 50 Ingots or masses of composite steels under my invention can be produced with facility either wholly or partially tubular in form, of such size, shape, and formation as required, by first inserting a tube of mild steel, either cast or welded, up as a core in the mold where- 55 in the first or center ingot is to be cast, then pouring the molten metal for the first ingot to

it. When it is designed to make an ingot wholly tubular, the center tube should project at either end, beyond the center and subsequent sections of the cast mass, so that when the mild steel comes to be cast around it the tube may not be inclosed, for by the pressure of the tube the mass may be forged with a ball or mandrel within it, securing more perfect results by the operation, the various portions of the final compound ingot or mass, made and prepared at the convenience and desire of the manufacturer, to be completed at any subsequent time, it being manifest that the article can be produced more cheaply and readily by using the steel-producing plant upon one quality at a time—that is, it would be more expensive to operate two sections of the producing-plant with a view of casting from both simultaneously metals of different qualities into the same ingot or mass. Not that I disclaim the mode of casting simultaneously, or nearly so, to produce the mass or ingot to be afterward submitted to the treatment of welding or re-fusing, but yet I do not think any necessity exists for such action, as it will not produce better, if equally good, results in the manufactured article, but will largely enhance the cost, producing an unsound article at the best, which unsoundness cannot be wholly removed by the subsequent treatment at the high welding temperatures because of the impurities and deleterious substances confined within the metals. When necessary, plates or slabs of mild steel, previously prepared by any process of reduction, can be used for the construction of the mold for receiving the steels, either in fluid or solid form and subsequent treatments. The aperture in such built-up mold must be closed so as to protect the high metals of the interior by metal stopper or cover capable of withstanding the necessary high heats. Sections of mild steel, either in plates, slab, or other form, may be used to cover an ingot or mass of steel already made, protecting the high metal during the subsequent treatment, and in all instances becoming a component part of the mass itself.

By my invention and mode of treatment, when it is desired to produce a perfect result from the combining of two or more qualities of steel, the surfaces of contact of any or all of the ingots, blocks, or masses, or sections thereof, should be freed from the presence of all impurities—as sand, scale, or slag—so that a free metallic surface is presented for union to the following metal. This will apply in all cases when a perfect result is to be obtained. The presence of sand, scale, or any deleterious substance confined within the metal will produce a weak spot or section which cannot be entirely overcome by subsequent working of the metal.

The cleansing process as a part of my invention is not an absolute requisite to the success of the process in all cases, for in many in-

stances the small amount of "dirt" confined would not seriously interfere with the practical results, yet for preciseness of metal, certain ability of all sections to do equal work, 5 the deleterious substances must be removed; preferably by acid baths, use of scraper, wire brush, or other means to produce the result of an unalloyed metallic surface. By my invention the ingots, blocks, or masses of composite steels may be formed in casting of such section, regular or irregular, as required, or with re-enforced portions, either in all the different sections of steels, or in any one of the 10 number composing the mass—as, for instance, in casting ingots, blocks, or masses for large shafts, the sections for wheel-seats, bearings, &c., can be enlarged either in any one or all the various steels composing the mass. This 15 is particularly applicable to the manufacture 20 of ordnance.

My invention contemplates the manufacture and production of compound or composite steels of two or more qualities, of any form and dimension, either solid, tubular, or partially so, with enlarged or reduced sections 25 the various sections formed by casting, using by preference the prior sections in a cold state, when casting another section to them any cracking or imperfections arising from the 30 shrinkage of the newly-poured metal upon a solid body, subsequently rectified by the process of welding, fusing, and manipulation while in such state of high heat, the various sections of the final ingot or mass to be cast, 35 cleansed, and prepared for the subsequent operation at the convenience of the producer, and by heating the mass entire, or in section, to the welding-heat of the exterior of mild steel, thereby securing the fusion or semi-fusion 40 of the mass of steels composing the ingot, slab, or bloom, producing soundness of the product in its entirety, the fusing of the different qualities together, and the perfect and complete union of the same.

45 It is a pretty-well known fact that steel which is high in carbon has a fusing-point which is lower than steel which is less high in carbon; or, in other words, that high steel is more fusible than low steel. It is also a well-known fact that in the presence of atmosphere 50 at the temperature of fusion carbon tends to burn out from the steel, and more rapidly from high steel at its low-fusing temperature than from low steel at its high-fusing temperature. 55 It is also a fact that the welding temperature of high steel is very close to its fusing-point, and that the burning-point of high steel in the presence of atmosphere is at or about perhaps a little lower than its welding-point. It is 60 therefore necessary to completely cover the surfaces which would otherwise be exposed to the atmosphere with the mild steel, and in case of tubular articles or hollow articles they should be surfaced with mild steel on both 65 sides in and out. It is also a known fact that the hammering or working of high steel is de-

sirable to give it toughness and bring out all the best qualities of the metal. This can only be done while its surface is protected.

The formation of an ingot of two or more qualities of steel arranged in layers is not of itself novel; but the formation of an ingot having on every side mild steel and on its interior higher steel, and then working that ingot under the hammer or in the rolls at a welding-heat, so to produce from the extreme exterior of the metal to the point of highest carbonization a gradual and comparatively uniform gradation of points of carbon is, so far as known, entirely novel. From these considerations it will be seen that at the welding-heat of the mild enveloping steel the high steel in the interior of the ingot will necessarily be in a state of fusion, so that the high steel is rolled or hammered while fused, and receiving this work the porosity of the metal is necessarily entirely removed. Some of its carbon diffuses undoubtedly into the adjacent mild steel, but not sufficient to materially change the quality of the exterior, and this change from high steel 90 to low steel is a gradual and progressive change, and not a sudden one, as it would be if the welding-heat were not given after the ingot had been poured.

The product of my invention will be of the 95 greatest utility to the public because of its cheapness and adaptability to most purposes for which iron and steel are now used, among which the more notable may be mentioned: ordnance and projectiles therefor, gun-carriages, armor, ship, boiler, and girder plate, railroad and street-road rails, frogs and switch-plates, shapes and bars for structural purposes, shafts and axles, both tubular and solid, tubes cast or welded, cylinders for hydraulic and 100 steam purposes, materials for construction of engines and cars, wire, tires for engine and car wheels, sheets, bars, and shapes for general or special use.

In the drawings, Figure 1 represents in end 110 elevation and section a composite steel plate made by my process, in which C is the outer envelope of mild steel and B the inner body of steel of higher carbon. Fig. 2 is a side elevation and section of the plate in Fig. 1. Fig. 3 115 represents a composite steel plate consisting of steels of three carbons—namely, the outer enveloping steel, C, the second steel, B, and the third steel, A. The inner steels may have any extent of carbon, and may be arranged in relation to each other as desired. Fig. 4 represents in horizontal section, and Fig. 5 in cross-section, a portion of a breech-loading gun made of composite steels, in which the portions C are of mild steel and the portions D E of steels 120 of higher carbon. Preferably, the steel D is of higher carbon than steel E. Fig. 4 also illustrates the re-enforcing referred to in the specification by increasing the relative thickness of the various carbon steels.

I am aware that Letters Patent No. 188,458, dated March 11, 1877, No. 213,256, dated April

1, 1879, and British Letters Patent No. 1,028, dated March 9, 1877, and No. 5,014, dated June 7, 1879, describe certain methods of forming and working composite steels; but I consider that they do not embrace the spirit of my invention.

Having thus fully described my invention, I claim and desire to secure by Letters Patent of the United States—

10 As a process for the manufacture of steel shapes, the two following manipulations: first manipulation, the formation of the ingot by

casting from converters or hearths of two or more different qualities of steel in a manner that shall leave the steel of high and hard quality enveloped in the steel of low or soft quality; second manipulation, forging, rolling, or working this composite ingot at the welding-heat of the mild steel; substantially as and for the purposes described.

JNO. J. WILLIAMSON.

Witnesses:

F. F. RAYMOND, 2d,  
WILLARD C. FOGG.